

April 21, 1925.

1,534,318

W. HOOPES ET AL

## ELECTROLYTIC REFINING OF ALUMINUM

Filed Dec. 21, 1922



Inventors  
W. HOOPES, F. C. FRARY  
and J. D. EDWARDS

By their Attorneys

Cooper, Ross & Dunham

## UNITED STATES PATENT OFFICE.

WILLIAM HOOPES, OF PITTSBURGH, AND FRANCIS C. FRARY AND JUNIUS D. EDWARDS, OF OAKMONT, PENNSYLVANIA, ASSIGNORS TO ALUMINUM COMPANY OF AMERICA, OF PITTSBURGH, PENNSYLVANIA, A CORPORATION OF PENNSYLVANIA.

## ELECTROLYTIC REFINING OF ALUMINUM.

Application filed December 21, 1922. Serial No. 608,285.

*To all whom it may concern:*

Be it known that we, WILLIAM HOOPES, FRANCIS C. FRARY, and JUNIUS D. EDWARDS, all citizens of the United States of America, the said WILLIAM HOOPES residing at Pittsburgh, and the said FRANCIS C. FRARY and JUNIUS D. EDWARDS residing at Oakmont, all in the county of Allegheny and State of Pennsylvania, have invented certain new and useful Improvements in Electrolytic Refining of Aluminum, of which the following is a full, clear, and exact description.

This invention relates generally to the refining of aluminum by electrolytic removal or separation of the metal from an alloy or a mixture thereof with other substances, and relates more particularly to a refining process in which the electrolyte floats, in a molten state, upon the molten alloy, the latter being used as anode and the aluminum removed being deposited on a layer of molten aluminum as cathode floating on the electrolyte.

In an extensively used aluminum reduction process, wherein aluminum is produced by reduction of its oxid, a cryolite bath or electrolyte is used, but in the herein described process, in which it is desired to have the refined metal float on the electrolyte, such a bath, though otherwise operable, cannot be used alone for the purpose, since in the molten state it is lighter than aluminum and hence would allow the latter to sink. While other salts may be added to give adequate density, such addition easily leads to difficulties of various sorts, resulting in failure to produce pure metal, and no prior inventor, so far as we are aware, has attained commercial success in this way or in any other. We have found that success may be realized and a bath produced combining the desired characteristics of density, fluidity, stability, capacity for dissolving alumina, conductivity, and selective solution and deposition of aluminum during electrolysis, by adding to cryolite (or preferably to a mixture of aluminum and sodium fluorids richer in aluminum fluorid than is cryolite) salts of the alkali earth metals. These metals are less easily precipitated from the bath than aluminum and we find

certain of their salts to be the only generally available material suitable for the purpose of increasing the density of the bath. We find that the only materials giving in high degree the other necessary or desirable characteristics are the fluorids of these metals (barium, strontium, calcium and magnesium). These form with cryolite, mixtures which are readily fusible, but our experience indicates that magnesium fluorid has less effect than any of the others in increasing the density of the bath. Barium fluorid has been suggested as an ingredient of electrolytes for other purposes, but so far as we are aware no one has heretofore suggested their use for refining aluminum or has given, with respect to the properties of barium fluorid and cryolite mixtures, the information needed for their successful use. We have found, however, that within certain limits, mixtures of the substances mentioned furnish excellent electrolytes, and that such a bath does not lose aluminum fluorid by volatilization at the working temperature to a serious extent. Its electrical conductivity and power of dissolving alumina are also good.

Moreover, the use, in an electrolyte, of a halogen salt other than a salt of fluorin, is in general disadvantageous and in some cases impractical. This is especially true in processes designed to produce substantially pure aluminum, for the reason that chlorids in the bath cause solution and deposition of other substances than aluminum, as for example zinc, iron, titanium, copper, and silicon, with the result that if the anode contains any of these substances the cathode metal may be contaminated therewith to an intolerable degree. Stated otherwise, if chlorin anions are present in the bath, it is difficult and in some cases impossible to prevent the solution of other substances than aluminum from the anode and their deposition on the cathode. On the other hand the presence of oxygen anions is permissible. Accordingly an advantageous feature of the present process is the use of a bath or electrolyte which may contain fluorin or oxygen anions or both but is substantially devoid of chlorids, and which therefore, as our experience shows, exerts a

truly selective action upon the anode alloy in dissolving aluminum therefrom substantially to the exclusion of other metals under conditions where it would be expected that 5 considerable amounts of other metals would be dissolved, and where, if substantial amounts of chlorides are present, they do actually dissolve.

We have determined the density of aluminum of 99.75 per cent purity to be approximately 2.29 grams per cc. at 1000° C. At this temperature, the density of molten cryolite is approximately 2.10 grams per cc. In order to increase the density of the cryolite, so that this aluminum will float on it at the temperature mentioned, we have found that there must be added about 20 parts of barium fluorid to each 80 parts of cryolite. If calcium fluorid were to be used, 10 about 40 parts would be required to 60 parts of cryolite. While the above mentioned mixture of cryolite and barium fluorid is completely molten at temperatures above 965° C., mixtures of calcium fluorid and cryolite containing about 40 per cent or more of the former by weight require a temperature above 1000° C. to keep them molten. This would make the working temperature 15 of the bath undesirably and in some cases impractically high. On the other hand, mixtures of cryolite and one or more fluorids of alkali earth metals having atomic weights above 80 are in general suitable; though of course radium is to be excepted, for obvious 20 reasons. Thus mixtures of cryolite and barium fluorid containing between about 20 and 60 per cent of the latter constituent by weight are readily fusible at temperatures below 1000° C., and have densities in the molten state ranging between about 2.38 and 25 3.15 grams per cc. at 1000° C. Even the heaviest of these mixtures is sufficiently light to float on any of a number of molten aluminum alloys suitable for use as anode in the 30 electrolytic refining of aluminum.

A fused mixture of cryolite and strontium fluorid containing between about 20 per cent and 60 per cent of the latter also lies within the proper range of densities for 35 our purpose, but such mixtures containing more than about 40 per cent of strontium fluorid are in general not so readily fusible as mixtures containing corresponding amounts of barium fluorid.

In operating with a bath of the type described above, it has been observed that there is a considerable deposition of metallic sodium at the cathode, and that this sodium, being in vapor form, passes up through the 40 molten aluminum cathode and causes difficulties in connection with the leading out of the current from the cathode metal. Carbonaceous rods used to carry the current out of the floating layer of aluminum are attacked and eventually disintegrated by the

sodium, but it has been found that this difficulty may be decreased, without interfering seriously with the density of the molten bath, by increasing the proportion of aluminum fluorid as compared to sodium fluorid, 70 although such an increase does perceptibly increase the electrical resistance of the bath.

As an example of baths or electrolytes which have been found by actual use to be suitable for our purpose, we recommend one 75 having approximately the following composition:

|                                                                    |                   |
|--------------------------------------------------------------------|-------------------|
| Barium fluorid                                                     | 30 to 38 per cent |
| Sodium fluorid                                                     | 25 to 30 per cent |
| Aluminum fluorid                                                   | 30 to 38 per cent |
| Alumina                                                            | 0.5 to 7 per cent |
| Calcium and magnesium fluorids (present as unavoidable impurities) | about 2 per cent  |

Such a bath is completely molten at all temperatures above about 900° C. and enables the refining to be carried on at about 90 950° C. At this temperature the bath is satisfactorily stable, has good electrical conductivity and satisfactory density, and is capable of dissolving a satisfactory amount of alumina.

It will be understood that the sodium and aluminum fluorids of the electrolyte may be supplied, in part at least, by cryolite, which has a composition generally accepted as  $3\text{NaF} \cdot \text{AlF}_3$ .

It has been observed that the density of these molten baths decreases more rapidly with rising temperature than does the density of the molten aluminum, and hence it is advantageous to provide a distinct margin of safety between the two densities, so that if the cell should become overheated the bath will not become so light as to permit the aluminum top layer to sink to the bottom. The density of bath of the above mentioned composition lies between about 2.5 and 2.7 at 950° C., and between about 2.4 and 2.6 at 1100° C., and accordingly pure aluminum will float on the bath at these temperatures, since the density of aluminum at 950° C. is about 2.30 and at 1100° C. is about 2.26 grams per cc.

A bath containing cryolite and 60 per cent of barium fluorid (instead of the chlorid) will dissolve between 4 and 5 per cent of alumina; and a similar bath containing 40 per cent barium fluorid, which would have a specific gravity of about 2.73, will dissolve between 8 and 9 per cent of alumina at 1000° C. Electrolytes of such type are therefore advantageous for the following reasons.

Alumina becomes more soluble in any of the cryolite baths as their temperature is raised, but if alumina be added until the bath is saturated it will be found that a small drop in temperature will cause some

of the alumina to precipitate out as corundum or in corundum-like form, with which more or less bath will be mechanically associated. In an operating cell the portion of the bath adjacent to the walls, together with that portion forming the top crust or coming in contact with it, is usually at a temperature distinctly lower than that of the main body of the bath, so that if sufficient alumina enters to saturate this main body the natural circulation will cause a deposition of part of the alumina on the walls of the cell in the form of a thickened crust. Practical operation of such a bath has shown that when the alumina has once crystallized in this form, it is extremely difficult to re-dissolve it in the bath. A certain amount of such crust on the interior of the cell is desirable for its thermal and electrical insulating properties (as described more fully in the copending application of William Hoopes, Junius D. Edwards and Basil T. Horsfield, Serial No. 608,289, filed December 21, 1922); but to prevent the formation of an undesired amount of this deposit, which would otherwise gradually fill up the cell and interfere with the operation, it is important to keep the alumina content below the saturation point. In order to maintain this condition it is therefore desirable, in practice, to have the bath capable of dissolving considerable alumina, so as to allow for unavoidable variations incident to operating conditions; for the reason that any of the following causes may operate to add alumina to the bath: (A) The hydrolysis of aluminum fluorid by moisture. Capillary action continually brings some of the bath up between the top metal layer and the side of the cell, so that it forms a crust on the top of the metal, where it is maintained at a high temperature and exposed to the air. The excess of bath above that which can solidify to form this crust drips back through the metal from time to time, and when the crust is disturbed or broken, parts of it sink through the metal, and return to the main body of the bath. (B) The reaction of sodium oxid (or hydroxid) with aluminum fluorid. More or less sodium is always liberated at the cathode, and some of it rises through the metal layer, probably in the form of vapor, and reaches the top crust where it is oxidized by contact with the air. (C) Direct oxidation of the floating aluminum layer by air penetrating through cracks in the top crust. (D) Alumina dust, which is always present in a plant in which the Hall process of producing aluminum is operated, will settle on the crust of the refining cell if it is operated in the same plant.

So important is it to have the bath unsaturated that in actual commercial operation it is generally necessary to remove

alumina from time to time. This may be conveniently done in various ways, as by one or another of the methods described and claimed in a copending application of William Hoopes and Francis C. Frary.

70

The cell preferred for use in our aluminum refining process is of the type described and claimed in the copending application of William Hoopes, Serial No. 608,287, filed December 21, 1922. One form of this cell is illustrated in the drawings annexed here-to, in which—

75

Fig. 1 is a plan view of the cell.

Figs. 2 and 3 are cross sections on lines 2—2 and 3—3, respectively, of Fig. 1.

80

Figs. 4 and 5 are detail cross sections on lines 4—4 and 5—5, respectively, of Fig. 1, illustrating the water connections to and from and between the water jackets.

Fig. 6 is a detail cross section on the line 6—6 of Fig. 1, showing the method of connecting the upper electrodes to the negative busbars.

85

Fig. 7 is a detail cross section on the same plane as Fig. 2, illustrating the method of securing the upper and lower shell sections together to give adequate mechanical strength without connecting the two electrically.

90

The lower shell or shell section 10 is preferably made of steel in the form of a cylindrical vessel of considerably greater diameter than height, and at or near its top it is provided with a water jacket 11 which is most conveniently formed by providing at the upper edge of the shell section an outwardly extending flange 12 of suitable width, and a flaring or conical ring 12<sup>a</sup> welded or otherwise hermetically joined to the underside of the flange and to the body 100 of the shell below.

95

Above the lower shell section 10 is an upper shell section 13 which may also be of steel and formed with hollow walls to provide an upper water jacket 14. The inner 110 surface of the upper shell section is preferably flaring, as indicated. To keep the sections electrically insulated or separated from each other a flat ring or gasket 15, of asbestos or other suitable material, may be used between the two.

105

In order to give the shell structure sufficient mechanical strength the sections may be secured together by means of machine studs 16 passing upwardly through the flange 12 and threaded into pads 17 welded on the bottom of the upper shell inside the water jacket. To prevent electrical connection the holes in the flange 12, through which the studs pass, may have insulating bushings 18 and insulating washers 19 may be used. If the water jackets are used, as in most cases they will be, the bushings and washers will not be subjected to a high temperature and hence they can be made of

115

120

125

130

practically any insulating material which will not soften at temperatures below 100° C. and which can withstand the crushing stress exerted by the studs. Mica has been 5 found to answer the purpose very satisfactorily.

Suitable water connections for the water jackets are provided, and for the sake of simplicity and convenience these connections 10 may be so constructed and arranged that the water flows through the two jackets in succession, preferably through the lower jacket first. For this purpose the jacket 11 may be provided at the bottom with an inlet nipple 15 20 connected by a pipe 21 to any convenient source of water, not shown, and at the top (to prevent pocketing of air) with an outlet nipple 22 connected by a pipe 23 to the inlet nipple 24 by which water from the 20 lower jacket is led into the bottom of the upper. The latter is equipped with an outlet nipple 25 (at the top to prevent air pocketing) which may be connected to a waste pipe 26 by means of a pipe 27. To 25 avoid electrical grounding the pipes 21 and 27 may consist of rubber hose, as may also the pipe 23 to keep the two shell sections electrically separate. The water used when the jackets are connected should be of sufficient 30 purity to prevent material flow of current from one shell section to the other at the voltage employed in operation.

In the bottom of the lower shell section a 35 layer 28 of heat-insulating material may be provided, as powdered bauxite, alumina, magnesia, or refractory bricks, to decrease or minimize loss of heat through the bottom of the cell, and above this layer is a bottom lining 29 of refractory electrically conducting material, preferably carbon, and preferably having a cavity or depression in its upper portion to receive the alloy or other material to be refined. The bottom lining 40 can be conveniently and satisfactorily made 45 by tamping into the shell a mixture of tar, pitch and granular or powdered coke, at a temperature high enough to make the mass plastic, and placing the shell and contents in an oven in which the temperature is gradually raised, say to about 600° C., for the purpose of baking and solidifying the carbonaceous mass.

Good electrical connection may be provided 50 between the shell and its bottom lining 55 by means of metal collector plates 31, welded to the inner surface of the shell so as to be electrically and mechanically continuous therewith. These plates extend inwardly into the bottom lining, which is 60 molded around them. At the plane of the collector plates the shell may be provided on the outside with metal contact pads 32, preferably welded to the shell so as to be 65 mechanically and electrically continuous therewith, to which pads busses or busbars,

of copper, aluminum or other suitable metal may be bolted tightly in place. The busbars 70 may be in the form of long flat plates 33 embracing the lower shell section, with their ends brought out at one side of the cell for convenient connection to one terminal of a suitable source (not shown) of continuous or unidirectional current. During the refining operation these busses are connected to the positive terminal or pole of the source, 75 so that the current enters the cell at the bottom. The carbon bottom or bottom-lining, 29, constitutes what may for convenience be termed the lower electrode of the cell.

The upper electrode may be multiple, as 80 indicated, composed preferably of a suitable number of short thick rods 34 of graphite, arranged vertically and having copper or other metal rods 35 threaded or otherwise suitably secured to the tops of the electrodes. 85 These metal rods serve to support the upper electrodes and convey current to and from the same, and for this purpose they may be releasably and adjustably secured, as by means of clamps 36, to metal busbars 37 extending horizontally across the cell. For convenience of access to the graphite cylinders, for adjustment, replacement, etc., the busbars may be arranged at two or more different levels, as indicated, and may be supported on and secured to a plurality of legs 38 to form a rigid frame work. The latter may rest on the upper shell section, in which case they are insulated from the shell section, as by any convenient and suitable means, not shown.

It is recognized that, strictly speaking, the aluminum layer floating on the bath and the layer of alloy underlying the bath, are the upper and lower electrodes, respectively, but these layers are termed herein the cathode and the anode, and hence it is deemed permissible as well as convenient to refer to the graphic cylinders and the carbon bottom-lining, or their equivalents, as the upper and lower electrodes.

Metal or other molten material may be withdrawn from the upper portion of the cell through a tapping notch 39, which may be closed by means of any suitable refractory material. Molten metal or other material may be withdrawn from the lower port of the cell through a port or tapping hole 40, normally closed by means of a plug of dense charcoal or other suitable material.

On the inside of the cell is a side-lining 45 extending upwardly from the carbon bottom 29, over the joint between the shell sections and well up toward or even over the top of the upper shell section. In practically all cases this side-lining should be thermally and electrically insulating, to decrease or minimize the conduction of heat 125 to the water jackets as well as to prevent by 130

passing of current around any part of the cell contents undergoing electrolytic treatment in the refining operation. The lining should be refractory enough to remain solid 5 at the temperatures to which it is exposed in the electrolytic refining operation. Under these conditions a lining composed of or formed from a mixture of metal fluorids and alumina, as more fully explained in the 10 copending application of William Hoopes, Junius D. Edwards, and Basil T. Horsfield, Serial No. 608,289, filed December 21, 1922, has been found highly satisfactory in practice.

15 In the refining process the aluminum alloy or mixture of aluminum and other substances lies in molten form in the bottom of the cell as indicated at 46. Floating on this is a layer 47 of fused bath or electrolyte, and 20 on the latter is a layer 48 of molten aluminum, with the upper electrodes extending into it far enough to insure good electrical contact. The molten layers are preferably established in the cell by successively pouring 25 the previously fused materials into place, using for the original aluminum layer the purest metal conveniently available. The cell may also be put in operation in the following manner.

30 The upper electrodes are lowered into contact with the carbon bottom and current is sent through them to the latter, thereby generating heat and fusing a small quantity of powdered or granulated bath material 35 placed around them. The upper electrodes are raised as the melting proceeds, and additional bath material is supplied, until a sufficient body of fused electrolyte has been produced. The molten anode alloy or mixture is then poured in. Almost any aluminum alloy can be used which is denser than the molten bath and which will remain mobile during the refining operation. Preferably, however, we use an alloy of which the 40 principal components are aluminum and copper. The alloy should be supplied in sufficient amount so that it will remain in an electrically continuous layer on the bottom of the cell throughout the refining operation.

45 A bath layer of sufficient depth should be used so that the top metal (the pure aluminum) will in no case come into contact with any portion of the side crust which has previously been covered by the anode alloy. It 50 is to be noted in this connection that the changes in composition of the anode alloy, incident to the refining operation, cause corresponding changes in its volume and in the position of the upper and lower surfaces of 55 the bath layer. Molten aluminum, preferably the purest obtainable, is placed on the molten bath, to serve as cathode.

The refining process can now be begun, with the alloy as anode and the top metal as 60 cathode, the current being led from the

top metal by means of graphite electrodes dipping into it. Under these conditions aluminum is dissolved out of the anode alloy and deposited in molten form on the cathode. This is continued until the desired amount of aluminum has been removed from the anode and added to the cathode. A portion of the top metal is then removed and the impoverished anode alloy is withdrawn through the tap hole 40, 70 fresh anode alloy in the molten state being supplied in any convenient way, preferably such that the refined metal floating on the bath will not be contaminated. This operation may be conveniently performed by 75 means of a carbon funnel, which after being preheated, is let down until it nearly reaches the bottom of the cell, which has preferably been cut out of the circuit. The refined metal entrapped in the funnel may 80 be dipped out with a hand ladle, after which the fresh anode alloy is poured in. The funnel is then lifted out and the refining process resumed. The fresh anode alloy introduced is preferably sufficient in amount 85 to raise the bath and top metal until the surface of the latter is at the same level as before the withdrawal. These operations may be repeated from time to time as necessary or desirable without seriously interrupting the refining process, which otherwise can go on continuously.

90 The energy-efficiency in electrolytic processes of refining aluminum is dependent largely upon the perfection of the measures taken for preventing escape of heat. Theoretically almost no energy is required for the refining; but practically, in the absence of some other adequate source of heat, sufficient electrical energy must be expended to maintain the anode, the bath, and the cathode in a fused condition, and consequently the amount of electrical energy which must be supplied is almost exactly 95 the equivalent of the heat permitted to escape. After the heat insulation of the cell has been perfected to the maximum practicable extent, nothing further can be accomplished in limitation of the amount of 100 heat escaping from a heated body of given dimensions, and with the minimum heat-loss the energy input required by the cell will also be a minimum. In the interests of power economy the cell should be operated at the lowest practicable voltage. Accordingly the electrolyte, which furnishes the major portion of the resistance, should be in as thin a layer as is permissible, and it has been found that a layer from 2½ to 105 4 inches thick is in general satisfactory. With a bath or electrolyte of any predetermined workable depth, the current density permissible varies between a lower limit 110 which is sufficient to maintain the anode, the bath and the cathode in a molten state. 115

and an upper limit at which volatilization of the bath is excessive or at which too large a proportion of anode impurities go into solution. These limits, with the various 5 bath-compositions which we have found satisfactory, are approximately 800° C. and 1100° C., respectively, with a preferable working temperature of about 950° C. Other miscible lower limit of current density also depends to a considerable extent 10 upon the size of the cell, since the ratio of area to volume is less in a large cell than in a small one.

In a cell having a cross section through 15 the electrolyte of 9.6 square feet it has been found that the preferable current is, in general, 8500 amperes, but that the process is workable with currents between 7500 and 12000 amperes. The preferable current 20 density in a cell having the electrolyte cross-sectional area mentioned is therefore 885 amperes per square foot, with a permissible minimum of about 780 amperes and a permissible maximum of about 1250 amperes, 25 per square foot. With the preferred current density mentioned, the total voltage between the terminals of the cell may be about 6 volts. Larger cells may be operated with lower current densities and at lower volt- 30 ages, and by varying the size of the cell, the composition of the bath, the conductivity of the bath, and the effectiveness of the heat insulation, the present electrolytic refining process is workable commercially with current densities between about 500 and about 35 2500 amperes per square foot of cross section of the bath. In general the lower practicable limit of voltage is about 3.5 volts and the upper limit is of course indefinite. 40 The current is led from the molten aluminum cathode preferably by means of the electrodes or current-carrying members described in the copending application of Francis C. Frary, Serial No. 672,867, filed 45 November 5, 1923. These are made of graphite, in the form of short, thick rods or cylinders, and may be protected against oxidation in the air by means of a non-oxidizable coating which may consist of molten 50 bath material applied to the rods as a thin layer and allowed to freeze thereon.

It is to be understood that the invention is not limited to the details herein specifically illustrated or described but can be carried out in other ways and with other apparatus, without departure from its spirit. 55 In the appended claims the expression "fluorid of an alkali earth metal having an atomic weight greater than 80," is used in a generic sense to include either barium or strontium fluorid or both, each of these metals having an atomic weight greater than that named. Similarly, in the claims specifying barium fluorid it is to be understood 60 that for a part of such fluorid, strontium

fluorid may be substituted in suitable proportion.

We claim—

1. In the electrolytic refining of aluminum, the steps comprising establishing between a lower layer of molten metal containing aluminum, as anode, and an upper layer of molten aluminum as cathode, an intermediate layer of molten electrolyte of greater density than the molten aluminum 75 and composed essentially of fluorids and substantially free from chlorid, and passing current from the anode metal through the electrolyte to the aluminum cathode whereby aluminum is removed from the anode 80 metal and deposited in the molten state on the cathode.

2. In the electrolytic refining of aluminum, the steps comprising establishing between a lower layer of molten metal containing aluminum, as anode, and an upper layer of molten aluminum as cathode, an intermediate layer of molten electrolyte of greater density than the molten aluminum 85 and composed essentially of fluorids and substantially free from other compounds except oxid, and passing current from the anode metal through the electrolyte to the aluminum cathode whereby aluminum is removed from the anode metal and deposited 90 in the molten state on the cathode.

3. In the electrolytic refining of aluminum, the steps comprising establishing between a lower layer of molten metal containing aluminum, as anode, and an upper layer of molten aluminum as cathode, an intermediate layer of molten electrolyte containing aluminum and sodium fluorids and between 20 and 60 per cent, approximately, 105 of fluorid of an alkali earth metal having an atomic weight greater than 80; and passing current from the anode metal through the electrolyte to the aluminum cathode whereby aluminum is removed from the anode metal 110 and deposited in the molten state on the cathode.

4. In the electrolytic refining of aluminum, the steps comprising establishing between a lower layer of molten metal containing aluminum, as anode, and an upper layer of molten aluminum as cathode, an intermediate layer of molten electrolyte substantially free from chlorid and containing aluminum and sodium fluorids and between 20 and 60 per cent, approximately, 115 of fluorid of an alkali earth metal having an atomic weight greater than 80; and passing current from the anode metal through the electrolyte to the aluminum cathode whereby aluminum is removed from the anode metal 120 and deposited in the molten state on the cathode.

5. In the electrolytic refining of aluminum, the steps comprising establishing between a lower layer of molten metal contain-

ing aluminum, as anode, and an upper layer of molten aluminum as cathode, an intermediate layer of molten electrolyte containing aluminum and sodium fluorids and between 20 and 60 per cent, approximately, of barium fluorid; and passing current from the anode metal through the electrolyte to the aluminum cathode whereby aluminum is removed from the anode metal and deposited in the molten state on the cathode.

6. In the electrolytic refining of aluminum, the steps comprising establishing between a lower layer of molten metal containing aluminum, as anode, and an upper layer of molten aluminum as cathode, an intermediate layer of molten electrolyte substantially free from chlorid and containing aluminum and sodium fluorids and between 20 and 60 per cent, approximately, of barium fluorid; and passing current from the anode metal through the electrolyte to the aluminum cathode whereby aluminum is removed from the anode metal and deposited in the molten state on the cathode.

7. In the electrolytic refining of aluminum, the steps comprising establishing between a lower layer of molten metal containing aluminum as anode, and an upper layer of molten aluminum as cathode, an intermediate layer of molten electrolyte containing between 20 and 60 per cent, approximately, of barium fluorid, and containing sodium and aluminum fluorids in such proportions that the ratio of aluminum fluorid to sodium fluorid is greater than cryolite; and passing current from the anode metal through the electrolyte to the aluminum cathode whereby aluminum is removed from the anode metal and deposited in the molten state on the cathode.

8. In the electrolytic refining of aluminum, the steps comprising establishing between a lower layer of molten metal containing aluminum, as anode, and an upper layer of molten aluminum as cathode, an intermediate layer of molten electrolyte containing cryolite, additional aluminum fluorid, and barium fluorid, the latter fluorid constituting between 20 and 60 per cent, approximately, of the whole; and passing current from the anode metal through the electrolyte to the aluminum cathode whereby aluminum is removed from the anode metal and deposited in the molten state on the cathode.

9. In the electrolytic refining of aluminum, the steps comprising establishing between a lower layer of molten metal containing aluminum, as anode, and an upper layer of molten aluminum as cathode, an intermediate layer of molten electrolyte substantially free from chlorid but containing between 20 and 60 per cent, approximately, of barium fluorid, and containing sodium and aluminum fluorids in such proportions that the ratio of aluminum fluorid to sodium

fluorid is greater than in cryolite; and passing current from the anode metal through the electrolyte to the aluminum cathode whereby aluminum is removed from the anode metal and deposited in the molten state on the cathode.

10. In the electrolytic refining of aluminum, the steps comprising establishing between a lower layer of molten metal containing aluminum, as anode, and an upper layer of molten aluminum as cathode, an intermediate layer of molten electrolyte substantially devoid of chlorid and containing cryolite, additional aluminum fluorid, and barium fluorid, the latter fluorid constituting between 20 and 60 per cent, approximately, of the whole; and passing current from the anode metal through the electrolyte to the aluminum cathode whereby aluminum is removed from the anode metal and deposited in the molten state on the cathode.

11. In the electrolytic refining of aluminum, the steps comprising establishing a lower layer of molten metal containing aluminum, as anode, and having a materially higher density than aluminum, an upper layer of molten substantially pure aluminum as cathode, and an intermediate layer of fused electrolyte composed of a suitable mixture molten at 1050° C., capable of dissolving a substantial amount of alumina, and having a density less than that of the anode metal but greater than that of the aluminum cathode metal; and passing current between the anode and the cathode.

12. In the electrolytic refining of aluminum, the steps comprising establishing a lower layer of molten metal containing aluminum, as anode, and having a materially higher density than aluminum, an upper layer of molten substantially pure aluminum as cathode, and an intermediate layer of fused electrolyte composed of a suitable mixture molten at about 950° C., capable of dissolving a substantial amount of alumina, and having a density less than that of the anode metal but greater than that of the aluminum cathode metal; and passing current between the anode and the cathode.

13. In the electrolytic refining of aluminum, the step comprising electrolyzing an impure aluminum-bearing molten metal or alloy of relatively high density as anode, with a superimposed molten bath containing cryolite and sufficient barium fluorid to give the bath a substantially higher density than aluminum and still permit the bath to dissolve a substantial amount of alumina.

14. In the electrolytic refining of aluminum, the step comprising electrolyzing an impure aluminum-bearing molten metal or alloy of relatively high density, as anode, with a superimposed molten bath substantially free from chlorid and containing cryolite and sufficient barium fluorid to give the

bath a substantially higher density than aluminum and still permit the bath to dissolve a substantial amount of alumina.

15. In the electrolytic refining of aluminum, the step comprising electrolyzing an impure molten aluminum-bearing metal or alloy of relatively high density as anode, with a superimposed molten bath containing aluminum, sodium, and barium fluorids, in proportions adapted to give the bath a greater density than that of aluminum and permit solution of a substantial amount of alumina.

16. In the electrolytic refining of aluminum, the step comprising electrolyzing an impure molten aluminum-bearing metal or alloy of relatively high density as anode, with a superimposed molten bath containing aluminum, sodium, and barium fluorids, in proportions adapted to give the bath a greater density than that of aluminum and permit solution of a substantial amount of alumina, the ratio of aluminum fluorid to sodium fluorid in said bath being greater than 25 in cryolite.

17. In the electrolytic refining of aluminum, the step comprising electrolyzing an impure molten aluminum-bearing metal or alloy of relatively high density as anode, with a superimposed molten bath containing barium fluorid between 30 and 38 per cent, sodium fluorid between 25 and 30 per cent, and aluminum fluorid between 30 and 38 per cent.

18. In the electrolytic refining of aluminum, the step comprising electrolyzing an impure molten aluminum-bearing metal or alloy of relatively high density as anode, with a superimposed molten bath of approximately the following qualitative and quantitative composition; barium fluorid between 30 and 38 per cent, sodium fluorid between 25 and 30 per cent, aluminum fluorid between 30 and 38 per cent, and alumina in amount less than sufficient to saturate the bath at the working temperature.

19. In the refining of aluminum, the step which consists in subjecting to electrolysis a combination of aluminum with a heavier metal in the molten state as anode, and substantially pure aluminum as cathode, said anode and cathode being gravitatively separated by an electrolyte containing cryolite and a heavy fluorid of a metal not more readily deposited than aluminum in amount sufficient to raise the specific gravity of the electrolyte without unduly decreasing its solvent power for alumina or its electrical conductivity, or increasing its freezing point.

20. In a process of electrolytically refining aluminum alloys with a fused electrolyte, compounding the electrolyte to give it a higher density than aluminum and a selective action in dissolving aluminum from the alloy.

21. In a process of electrolytically refining aluminum alloys with a fused electrolyte, compounding the electrolyte to give it a higher density than aluminum and a selective action in dissolving aluminum from the alloy, and depositing from said bath upon a suitable cathode, aluminum of a high degree of purity.

22. In a process of electrolytically refining aluminum alloys with a fused electrolyte, compounding the electrolyte so as to limit the production of sodium at the cathode.

23. In a process of electrolytically refining aluminum alloys with a fused electrolyte, wherein current-carrying means are employed in contact with the molten cathode, compounding the electrolyte to minimize the production at the cathode of substances which attack the current-carrying means, whereby the useful life of the latter is substantially prolonged.

24. In a process of electrolytically refining aluminum alloys with a fused electrolyte, wherein a molten anode, electrolyte, and cathode are arranged in gravitatively separated layers, with current-carrying means in contact with the cathode, compounding the electrolyte to limit the production at the cathode of substances which attack said current-carrying means, and to maintain the gravitational separation of said layers.

25. In a process of electrolytically refining aluminum alloys with a fused electrolyte, wherein a molten anode, electrolyte, and cathode are arranged in gravitatively separated layers, compounding the electrolyte to limit the production of sodium at the cathode and maintain the gravitational separation of said layers.

26. In a process of electrolytically refining aluminum alloys with a fused electrolyte, wherein a molten anode, electrolyte, and cathode are arranged in gravitatively separated layers, compounding the electrolyte to limit the production of sodium at the cathode and give the electrolyte a selective action in dissolving aluminum from the anode, and a density adapted to maintain the gravitational separation of said layers.

27. In a process of electrolytically refining aluminum alloys with a fused electrolyte, limiting the introduction of oxygen into the electrolyte by compounding the electrolyte so as to limit the production of metallic sodium at the cathode.

28. In a process of electrolytically refining aluminum alloys with a fused electrolyte, compounding the electrolyte to give the same, when fused, a greater density than molten aluminum at the same temperature and to remain fluid at permissible working temperatures without excessive volatilization.

29. An electrolyte composition for the purpose described containing aluminum and

sodium fluorids, and between 20 and 60 per cent, approximately, of fluorid of an alkali earth metal having an atomic weight greater than 80.

5 30. An electrolyte composition for the purpose described, substantially free from chlorid, containing aluminum and sodium fluorids, and between 20 and 60 per cent, approximately, of fluorid of an alkali earth metal having an atomic weight greater than 80.

10 31. An electrolyte composition for the purpose described composed essentially of fluorids and substantially free from other compounds except oxid, and containing aluminum and sodium fluorids, and between 20 and 60 per cent, approximately, of fluorid of an alkali earth metal having an atomic weight greater than 80.

15 32. An electrolyte composition for the purpose described containing aluminum and sodium fluorids and between 20 and 60 per cent, approximately, of barium fluorid.

20 33. An electrolyte composition for the purpose described containing aluminum and sodium fluorids and between 20 and 60 per cent, approximately, of fluorid of an alkali earth metal having an atomic weight

greater than 80, and less than about 2 per cent of fluorid of an alkali earth metal having an atomic weight below 80. 30

34. An electrolyte composition for the purpose described containing the following compounds in approximately the proportions named: aluminum fluorid 30 to 38 35 per cent, sodium fluorid 25 to 30 per cent, and barium fluorid 30 to 38 per cent.

35. An electrolyte composition for the purpose described containing aluminum and sodium fluorids and between 20 and 60 per 40 cent, approximately, of fluorid of an alkali earth metal having an atomic weight greater than 80, with less than about 7 per cent of alumina.

36. An electrolyte composition for the 45 purpose described containing the following compounds in approximately the proportions named: aluminum fluorid 30 to 38 per cent, sodium fluorid 25 to 30 per cent, and barium fluorid 30 to 38 per cent; with less 50 than about 7 per cent of alumina.

In testimony whereof we hereto affix our signatures.

WILLIAM HOOPES.  
FRANCIS C. FRARY.  
JUNIUS D. EDWARDS.